

1

2,780,511

**METHOD OF MAKING CELLULOSE ACETATE TEXTILE FIBERS BY ACETYLIZATION OF REGENERATED CELLULOSE FIBERS**

Takeso Takagi, Tokyo, Japan, assignor to Toho Rayon Co., Ltd., Tokyo, Japan, a corporation of Japan

No Drawing. Application May 14, 1953,  
Serial No. 355,150

3 Claims. (Cl. 8—121)

This invention relates to the preparation of cellulose acetate fiber having an acetic acid content of at least 40% by vapor phase acetylation of cellulosic fibers while retaining the fiber structure.

It has previously been proposed to acetylate cellulosic fibers while retaining their fiber structure by carrying out the acetylation both in liquid and vapor phase. However, it has hitherto been impossible to produce a cellulose acetate fiber having an acetic acid content from 40-62% by weight (which corresponds approximately to cellulose diacetate or triacetate) free from discoloration and brittleness and having at the same time a high tensile strength and low elongation. Direct acetylation of cellulose has hitherto generally been employed commercially to produce only cellulose monoacetate fiber, while fibers having a higher acetic acid content have been made commercially by complete acetylation followed by a dry spinning procedure involving partial hydrolysis to reduce the acetic acid content. In the first case, the acetate fiber is a mere modification of ordinary cellulose fiber possessing essentially the same chemical properties and dry affinity as ordinary cellulose. Dry spun cellulose acetate fiber on the other hand, even when the acetic acid content has been reduced to approximately that of cellulose diacetate, possesses undesirably low tensile strength and high elongation.

One object of the present invention is to provide a cellulose acetate fiber having an acetic acid content corresponding approximately to cellulose diacetate and cellulose triacetate and having a high tensile strength together with low elongation and essentially the same dyeing characteristics as dry-spun acetate fiber.

Another object is to provide a cellulose acetate fiber having a permanent structural crimp and having an acetic acid content from 40-62% by weight, preferably from 40-55% by weight.

Still a further object is to provide a process for continuous vapor phase acetylation of cellulosic fibers while retaining the fibrous structure of the cellulosic material.

A further object is to provide a method for the vapor phase acetylation of cellulosic fibers, particularly fibers of regenerated cellulose, while retaining the fiber structure, without discoloration of the fibers.

Other and further objects will be apparent from the description which follows.

The present invention may be employed for the production of cellulose acetate fibers from a wide variety of cellulose fibers, including cotton, regenerated cellulose and wood-pulp. However, the invention is particularly

2

advantageous when applied to the viscose staple rayon having a permanent structural crimp. This crimp, in contrast to the mechanically applied crimp of the thermoplastic fibers, originates in the fine inner structure of the fibers and is permanent through spinning, weaving, washing, ironing and other similar fabric treatments, which makes such viscose fiber particularly valuable. The permanent structural crimp of such viscose staple rayon is retained throughout the acetylation process of the present invention.

The invention may be applied to continuous cellulosic fibers which may be lightly twisted together to form a yarn or rope prior to acetylation, or it may be applied to a mass of loose staple fibers which may be conveyed through the several steps of the process on a suitable belt or wire mesh conveyor, or the like. If desired, the cellulosic fibers, either continuous or staple, may be loosely woven or knitted to form a fabric which may then be subjected to the acetylation process of the present invention.

The invention is characterized in that the cellulosic fiber is impregnated with an acetylation catalyst from an aqueous solution thereof, dried to remove at least a portion of the water content of the impregnated fiber, treated with acetic acid vapor to replace and remove the residual water content, then acetylated with acetic acid anhydride in vapor form. The entire process is preferably carried out with the cellulosic fiber advancing continuously through each successive step, particularly the steps involving treatment with acetic acid and with acetic anhydride.

Among the acetylation catalysts which are suitable for use in the present invention are salts, of which there are particularly preferred the acetates such as potassium, sodium, or lithium acetates; the phosphates, such as sec.-sodium phosphate, tert.-sodium phosphate, the ammonium phosphates, etc.; the chlorides, such as zinc chloride, cupric chloride, aluminum chloride, stannous chloride, stannic chloride, etc.; the sulfates, such as copper sulfate, aluminum sulfate, zinc sulfate, alum, etc.; and the oxalates, such as ammonium oxalate, ammonium acid oxalate, etc.; and mixtures of any two or more of such salts.

The catalysts are preferably applied to the cellulosic fiber from aqueous solution which may suitably contain from about 10-20% by weight of the desired salt. The fiber may be passed through a container filled with the aqueous salt solution or the solution may be sprayed onto the fibers, the impregnation preferably being carried out at room temperature (although elevated temperatures may be employed if desired) at which temperature a contact time of from about 10 to about 60 minutes is employed to insure satisfactory impregnation of the fiber. The impregnated fiber, which contains about 5-15% by weight of the catalyst, is then passed between squeeze rolls to remove excess water, or it may be centrifuged if desired, and further dried in hot air. The dried fiber ordinarily has a water content at this point of from 40-75% by weight, usually from 55-65% by weight.

In order to minimize the quantity of acetic anhydride that is required for the acetylation reaction, it is preferred to replace and remove the residual water content of the impregnated fibers following the aforementioned drying operation by passing the fibers continuously through a closed chamber filled with acetic acid vapor and main-

tained at a temperature of 100° to 130° C., preferably at a temperature of 105° to 115° C. Removal and replacement of residual water ordinarily is completed in from 10 to 45 minutes, the best results having been obtained in a period of about 25 to 35 minutes.

Immediately following the exposure to acetic acid vapor the fiber is advanced into a separate chamber filled with acetic anhydride vapor and maintained at about 100° to 140° C., preferably at about 110° to 130° C. In order to achieve the desired degree of acetylation the fiber must be maintained in contact with acetic anhydride vapor for a period of at least 3 hours, preferably from 4 to 7 hours, during which time the supply of acetic anhydride vapor to the reaction chamber is constantly renewed. The acetic acid present in the fiber as it is introduced into the acetylation chamber together with the acetic acid formed during acetylation reaction is constantly withdrawn along with the excess acetic anhydride vapor. The mixture is condensed and then distilled in a conventional stainless steel plate column to separate the anhydride from the acid. The anhydride is then recirculated to the acetylation chamber.

The acetylated fiber is continuously withdrawn from the acetylation chamber through a restricted opening, washed with water, oiled and dried.

The cellulose acetate fiber of the present invention has unexpectedly excellent physical properties as compared with the conventional dry-spun acetate fibers, having a dry tensile strength of at least 1.70 gram/denier, a wet tensile strength of at least 1.30 gram/denier, a loop tensile strength of at least 1.25 gram/denier, while having an ultimate elongation no greater than about 25% (dry) and about 22% (wet). The physical properties of the preferred fibers of the present invention having an acetic acid content of 40-55% by weight are even better. The dye affinity of the acetate fibers of this invention, on the other hand, is substantially the same as that of dry-spun acetate fiber, the fibers being dyed with celliton color and not with direct dyes, whereas cellulose monoacetate fibers made by fibrous acetylation are dyed with direct color and not with celliton color. In addition, the acetate fibers of the present invention have a lower moisture regain (not over 7.5%) than cellulose monoacetate fibers.

The following specific examples are given by way of illustration and are not intended as a limitation upon the scope of the invention.

#### Example I

Viscose rayon staple fiber having a permanent structural crimp (6.8 per cm.) is immersed in an aqueous solution containing about 15% sodium acetate for an hour at room temperature. The fiber is then dehydrated in a centrifuge to reduce the water content to approximately 100% of the weight of the fiber, the amount of catalyst contained in the fiber being then about 10% by weight of the fiber. The fiber is then picked and further dried in hot air to approximately 60% water content. The loose fiber is then placed on a wire mesh conveyor belt on which it is carried through a closed chamber maintained at about 110° C. and filled with acetic acid vapor at atmospheric pressure, the time of exposure of the fibers to the acid vapor being approximately 30 minutes. The fiber comes out of the acid chamber through a slit and is then advanced through a slit into a second closed chamber filled with acetic anhydride vapor at atmospheric pressure, the second chamber being maintained at a temperature of about 130° C. The fiber is allowed to remain in the second chamber for about five hours in order to reach the desired degree of acetylation, the acetic anhydride being vaporized from the lower portion of the chamber from a constantly renewed supply. The acetic acid carried into this chamber on the fibers, together with any acetic acid formed during the acetylation reaction is constantly removed from the chamber along with excess acetic anhydride vapor. The mixed vapors are then con-

ensed and separated by fractional distillation, the acetic anhydride recovered being returned to the acetylation chamber where it is revaporized.

After the desired degree of acetylation has been achieved the fiber, carried by the conveyor belt, is withdrawn through a slit in the chamber wall and is then washed with water, oiled and dried in air at 50°-70° C. The resulting cellulose acetate fiber retains the permanent structural crimp of the original viscose rayon fiber and has an acetic acid content of 52% by weight.

#### Example II

Spun-dyed viscose staple fiber having a permanent structural crimp is treated as described in Example I, except that an aqueous solution of potassium acetate is used in place of the sodium acetate solution, the amount of catalyst contained in the fiber being about 8% by weight of the fiber. The chamber containing acetic anhydride is maintained at a temperature of 120° C. and the time of exposure of the fiber to the acetic anhydride vapors is six hours. The resulting product has an acetic acid content of 53%, the acetylated fiber having the same permanent structural crimp as the original viscose staple fibers. The color of the original dyed viscose staple may be black, blue, brown, orange, yellow, navy blue, pink, purple, red, or any other color and the shade of these colors is not changed by the acetylation procedure.

#### Example III

30 Yarn made from viscose rayon staple fibers having a permanent structural crimp is treated as described in Example I, except that zinc sulfate is used as the catalyst and the acetylation is carried out for five hours at 130° C. The resulting cellulose acetate yarn having an acetic acid content of 50%, retains its original crimped fibrous structure.

#### Example IV

35 Spun-dyed viscose rayon yarn made from fibers having a permanent structural crimp is treated as described in Example I, except that 12% ammonium oxalate based on the weight of the yarn is employed as the catalyst. The resulting cellulose acetate yarn possesses the same color and crimped fibrous structure as the original viscose rayon yarn and has an acetic acid content of 49%.

#### Example V

40 Fabric woven from a viscose rayon yarn made from fibers having a permanent structural crimp is treated as described in Example I, except that 6% sec.-sodium phosphate based on the weight of the fabric is employed as the catalyst. The acetylation is carried out for six hours at a temperature of 110°-130° C. The resulting cellulose acetate fabric retains the crimped fibrous structure of the original fabric and possesses a 48% acetic acid content 45 while having good draping qualities and also a good hand.

#### Example VI

45 Fabric woven from spun-dyed viscose rayon staple fiber having a permanent structural crimp is treated as described in Example I, except that tertiary sodium phosphate is employed as catalyst, the acetylation being carried out at 110°-130° C. for five hours. The resulting cellulose acetate fabric possesses the same color and crimped fibrous structure as the original and has a 50% acetic acid content.

#### Example VII

50 Viscose rayon staple fibers having a permanent structural crimp are treated as described in Example I, except that the acetylation is carried out for four hours at 120° C. The resulting cellulose acetate fiber possesses the same crimped fibrous structure as the original fiber and has a 42% acetic acid content.

55 The superiority of the cellulose acetate fiber of the present invention as compared to cellulose monoacetate

made by fibrous acetylation or dry-spun acetylated fiber made by complete acetylation followed by partial hydrolysis is shown in the following table:

vapor at 100°-140° C. for a period of at least three hours.

2. The method as defined in claim 1 in which said re-

|                                | Monoacetate fiber                                                               | Products of the present invention                                                       | Dry-spun acetate fiber                                       |
|--------------------------------|---------------------------------------------------------------------------------|-----------------------------------------------------------------------------------------|--------------------------------------------------------------|
| Acetic acid content (percent)  | 29.                                                                             | 40.                                                                                     | 51.                                                          |
| Tensile strength (dry), g./d.  | 2.05.                                                                           | 1.90.                                                                                   | 1.48.                                                        |
| Tensile strength (wet), g./d.  | 1.45.                                                                           | 1.40.                                                                                   | 0.82.                                                        |
| Tensile strength (loop), g./d. | 1.40.                                                                           | 1.35.                                                                                   | 0.93.                                                        |
| Elongation (dry), percent      | 19.                                                                             | 15.9.                                                                                   | 26.0.                                                        |
| Elongation (wet), percent      | 21.                                                                             | 19.9.                                                                                   | 28.0.                                                        |
| Dye affinity                   | Same as cellulose fiber.<br>Dyed with direct color and not with cellulon color. | Same as dry-spun cellulose acetate. Dyed with cellulon color and not with direct color. | Dyed with cellulon color and not with direct color.          |
| Moisture regain (percent)      | 9.5.                                                                            | 7.5.                                                                                    | 5.6.                                                         |
| Number of crimp per cm.        |                                                                                 |                                                                                         | 6.8 (permanent structural crimp).<br>7.4 (mechanical crimp). |
| Crimp elasticity (percent)     |                                                                                 |                                                                                         | 69.8.<br>65.5.                                               |

It is apparent from the foregoing data that the fiber of the present invention differs in chemical structure and dyeing properties from the monoacetate fiber, being in these respects closely similar to the dry-spun acetate fiber, but possesses remarkably superior physical properties as compared to the dry-spun acetate fiber.

The process of the present invention makes it possible to produce cellulose acetate fibers having the same fiber structure as the starting material and having an acetic acid content approximately equal to cellulose diacetate or triacetate (40-62% by weight) without discoloration or staining of the fiber and without embrittlement. The invention also makes possible the production of such cellulose acetate products in a continuous process using a relatively small amount of acetylation catalyst without the necessity for carrying out the acetylation step at reduced pressures. Moreover, the fibers of this invention may be produced in the form of a loose mass, lap or roving, which, because of the excellent physical properties of the fibers, is admirably adapted for further processing into yarns, threads, and woven or knitted fabrics, or they may be produced in the finished form of yarns, threads, and woven or knitted fabrics directly from corresponding cellulosic yarns, etc. without loss of fibrous structure.

Although I have herein described specific embodiments of my invention, I do not intend to limit myself solely thereto, but to include all of the obvious variations and modifications within the spirit and scope of the appended claims.

I claim:

1. The method of making cellulose acetate textile fibers which comprises impregnating regenerated cellulose fibers with 5% to 15% by weight of an acetylation catalyst salt from an aqueous solution thereof, drying said impregnated fibers to remove a portion of the water from said impregnated fibers, replacing completely the residual water in said fibers with acetic acid by maintaining said fibers in contact with acetic acid vapor at 100°-130° C. for a period from 10 to 45 minutes and subsequently acetylating said fibers to an acetic acid content from 40% to 62% by weight while retaining their fibrous form by maintaining said fibers in contact with acetic anhydride

25  
30  
35  
40  
45  
50  
55  
60  
65

generated cellulose fibers are in the form of a loose mass of viscose rayon staple fibers having a permanent structural crimp.

3. The method of acetylating viscose rayon staple textile fibers having a permanent structural crimp which comprises impregnating said fibers with an acetylation salt catalyst from an aqueous solution containing about 10% to 20% of said catalyst to provide impregnated fibers containing about 5% to 15% of said catalyst by weight of the fibers, drying said impregnated fibers to reduce the water content thereof to 40% to 75% by weight, passing said fibers continuously through a chamber maintained at 100°-130° C. and filled with acetic acid vapor with said fibers in contact with said acetic acid vapor for 10 to 45 minutes until the residual water in said fibers has been completely replaced with acetic acid, and subsequently passing the fibers continuously through a chamber maintained at 110°-130° C. and filled with acetic anhydride vapor, the period of contact between said fibers and acetic anhydride vapor being three to seven hours, and continuously removing acetic acid vapor and excess acetic anhydride vapor from said last-named chamber until there is produced cellulose acetate fibers having a permanent structural crimp, an acetic acid content from 40% to 62% by weight, a dry tensile strength of at least 1.70 gram/denier, and a wet tensile strength of at least 1.30 gram/denier.

#### References Cited in the file of this patent

#### UNITED STATES PATENTS

|           |              |                |
|-----------|--------------|----------------|
| 1,823,350 | Clark et al. | Sept. 15, 1931 |
| 1,861,320 | Rheiner      | May 31, 1932   |
| 1,926,498 | Rheiner      | Sept. 12, 1933 |
| 2,253,724 | New et al.   | Aug. 26, 1941  |

#### FOREIGN PATENTS

|         |               |               |
|---------|---------------|---------------|
| 263,938 | Great Britain | Jan. 6, 1927  |
| 264,937 | Great Britain | Jan. 31, 1927 |
| 755,267 | France        | Sept. 4, 1933 |

#### OTHER REFERENCES

Matthews' Textile Fibers, 5th ed., May 1947, pages 800, 822, 825.  
Textile World, September 1949, pages 111-130.